

1

3,139,357

## PROCESS OF SUPPORTING AND COOLING SHAPE HOT METAL

William B. Arnold, Niagara Falls, N.Y., assignor to Great Lakes Carbon Corporation, New York, N.Y., a corporation of Delaware  
No Drawing. Filed Dec. 14, 1960, Ser. No. 75,675  
12 Claims. (Cl. 148—4)

This invention relates to a process for supporting shaped hot metal during its cooling period. More specifically, this invention relates to the supporting of hot metal, such as aluminum, magnesium and alloys thereof, after it has been formed, such as by extrusion.

In the extrusion of metals, such as aluminum, into rods or other desired shapes, it is conventional to heat the metal to a high temperature in order that it might be conveniently extruded or formed into the desired shape and size. After the forming step the article must be cooled for subsequent handling.

Graphite supports such as canisters and "run-out" tables have in the past been employed to assist in the cooling operation. These "tables" may be in the form of a series of rectangular blocks of equal thickness and typically are laid lengthwise for a distance sufficient to bring about substantial cooling of the formed metal by the time it reaches the end of the run-out table. The top surface of these blocks may be grooved in order to form a pathway for the metal. Graphite was chosen because of its ability to withstand high temperatures and at the same time absorb and dissipate heat readily. Another reason for its selection was its relative softness thereby assuring that it would not scratch the surface of the hot and frequently soft metal body sliding over or through it and being cooled.

However the employment of graphite for this purpose has one serious disadvantage and that is that the graphite marks or blackens the surface of the hot metal which contacts and slides along the graphite table or through canisters. This marking or blackening has brought serious objections from the metal purchasers. It has therefore frequently been necessary for the metal manufacturer to remove the objectionable marking from the metal. This has required a post-cooling cleaning step or other post-cooling processing and costly labor expenses in removing these marks from the aluminum.

This invention has as one of its objects the cooling and supporting of hot metal shapes by graphite and at the same time the substantial elimination of the aforesaid objectionable marking considered inherent when employing graphite for this purpose.

The invention has as an additional object the achievement of the foregoing in a convenient, economical and efficient manner.

It is a finding of this invention that the foregoing objectives may be obtained by subjecting graphite bodies such as previously employed for these purposes to a "post-forming" treatment. The graphite bodies which are subjected to this post-forming treatment will be of any desired shape, will be porous in nature and will typically have an apparent density between about 1.52 and about 1.60. The post-forming treatment consists in filling a substantial percentage of the pores of the graphite bodies with a material found capable of substantially eliminating the marking of the hot metal by the graphite. Many materials have been found to be suitable for this purpose and operative in the present invention. They may all be considered as waxy substances and are discussed in more detail hereinafter.

The waxy substance employed to occupy or fill the pores in the pre-formed graphite bodies may be processed

2

into the pores in several different ways such as by soaking the graphite body in the material for a sufficient length of time to obtain the desired pickup, impregnating the graphite body by using a normal vacuum-pressure cycle in an autoclave, or by impregnating in an autoclave by pressure alone. The impregnating material may be heated to liquefy it, if necessary, prior to these procedures. It may also be dissolved in a volatile solvent prior to same or it may sometimes be expedient to employ it as an aqueous emulsion. With any of these techniques, the desired pick-up is preferably from 6 to 12% by weight of solvent-free impregnant based on the weight of the graphite body with from about 3% to about 25% being operative.

Without in any way being bound by theoretical considerations it is believed that what occurs as the hot metal slides over the thus treated graphite is that the impregnating material continuously migrates by capillary action toward the surface of the graphite body which is contacted by the hot metal and thus forms a very thin film at this surface which prevents or minimizes actual contact between the metal and the graphite. The graphite body still therefore functions to dissipate the heat as desired but does not cause the objectionable marking of the hot metal as has previously been the case. The metal bodies being cooled are frequently at temperatures between 300 and 400° C. and generally below 500° C. The materials employed to occupy the pores of the graphite will typically be solid and have a melting point above 40° C. and preferably between about 60° C. and about 100° C. The temperature of the hot metal therefore is high enough to cause melting of the impregnating material at and near the surface of the graphite body which is contacted by the metal. When the impregnating material at or near the surface of the graphite body is raised toward the high temperatures of the metals being cooled, it either vaporizes away from the graphite body or melts away from the contacting surface. In either event it is replaced by what is believed to be capillary action, by some more of the impregnating material from the pores of the graphite body thereby constantly providing a thin film or barrier between the hot metal and graphite body.

Employing the impregnating materials in accordance with the teachings of this invention not only serves to reduce or eliminate the marking of the hot metal by the graphite, but also assists in reducing the friction between the graphite and the hot metal sliding over same. In other words it augments the lubricating action of the graphite. This is important in connection with cases where the metal bodies being cooled are malleable to a degree approaching limpness and where anything that obstructs or interferes with its smooth and even progress is apt to cause the extruded or formed work to be deformed. It is also important in the case of heavy extrusions, where a minimum amount of friction is desired.

The pre-formed porous graphite bodies which are subsequently impregnated may be made from artificial graphite or electrographite or may be formed from a mixture of ordinary coke or carbon particles and pitch and baked and graphitized in a conventional manner. In any case the bodies employed will be those which are porous and which have been pre-formed prior to the addition of the impregnating material. Mantell's volume on "Industrial Carbon," 2nd Edition, 1946, pages 268-270, and U.S. Patent 2,862,748 to Bailey et al., particularly column 3, lines 18-35, give additional details as to the making of such bodies and their typical characteristics.

The waxy substances employed to impregnate the pores of the graphite should be non-halogenated, should not flash into flame when raised to or toward the temperatures

of the metal bodies being cooled, and should not give off any obnoxious or harmful fumes when heated.

The waxy substances may be natural waxes among which are: mineral waxes such as paraffin wax, petroatum wax, ozokerite, ceresin, Utah wax and montan wax; vegetable waxes such as carnauba wax, flower wax, first wax, medium wax, sandy wax, fat wax, candelilla wax, Japan wax, Ucuhuba wax, Bayberry wax, Ouricury wax, cocoa butter, fiber wax, fir-bark wax, cotton wax, flax wax, sugar-cane wax and rice-oil wax; animal waxes such as spermaceti; and insect waxes such as beeswax.

The waxy substances employed may also be manufactured and synthetic waxes among which are: fatty alcohols such as cetyl alcohol, lanette wax, and stearyl alcohol; fatty acids such as stearic acid, palmitic acid and myristic acid; polyhydric alcohol-fatty acid esters such as glyceryl stearates, glycol fatty-acid esters and sorbitol stearates; and hydrogenated oils such as opalwax. Metal salts such as alkali and alkaline earth salts of the fatty acids may also be employed. The employment of mixtures of these materials is also contemplated. Several other suitable waxy materials may be found in Bennett's "Commercial Waxes," 2nd Edition, 1956, published by Chemical Publishing Co., Inc., 212 Fifth Avenue, New York, N.Y.

Although this invention has been illustrated by citing specific details embraced within the scope of the invention, it is to be understood that various modifications within the invention are possible, some of which have been referred to above. I therefore do not wish to be limited except as defined by the appended claims.

I claim:

1. A process of cooling and supporting solid, heated metal which comprises sliding said solid, heated metal in contact with preformed, porous graphite containing a material selected from the group consisting of waxes and metal salts of fatty acids in the pores thereof until a substantial amount of the heat of the metal has been dissipated by the graphite.

2. A process of cooling and supporting solid, heated metal which comprises sliding said solid, heated metal

in contact with preformed, porous graphite containing a wax in the pores thereof until a substantial amount of the heat of the metal has been dissipated by the graphite.

3. The process of claim 1 wherein the hot metal is aluminum.

4. The process of claim 1 wherein the graphite contains from about 3% to about 25% by weight of said selected material in the pores thereof.

5. The process of claim 2 wherein the wax is selected from the group consisting of mineral waxes, vegetable waxes, animal waxes, insect waxes and synthetic waxes.

6. The process of claim 2 wherein the melting point of the wax is at least 40° C.

15 7. In the process of cooling solid, heated metal by sliding said solid, heated metal in contact with graphite, the improvement which comprises employing preformed, porous graphite containing a material selected from the group consisting of waxes and metal salts of fatty acids in the pores thereof, thereby substantially eliminating any marking of the metal by the graphite.

20 8. In the process of cooling solid, heated metal by sliding said solid, heated metal in contact with graphite, the improvement which comprises employing preformed, porous graphite containing a wax in the pores thereof, thereby substantially eliminating any marking of the metal by the graphite.

25 9. The process of claim 7 wherein the hot metal is aluminum.

30 10. The process of claim 7 wherein the graphite contains from about 3% to about 25% by weight of said selected material in the pores thereof.

11. The process of claim 8 wherein the wax is selected from the group consisting of mineral waxes, vegetable waxes, animal waxes, insect waxes and synthetic waxes.

35 12. The process of claim 8 wherein the melting point of the wax is at least 40° C.

#### References Cited in the file of this patent

#### UNITED STATES PATENTS

1,010,237 Conniff ----- Nov. 28, 1911  
2,333,387 Parvin ----- Nov. 2, 1943